

# UNITED STATES PATENT OFFICE.

CLARENCE I. B. HENNING, OF WILMINGTON, DELAWARE, ASSIGNOR TO E. I. DU PONT DE NEMOURS & COMPANY, OF WILMINGTON, DELAWARE, A CORPORATION OF DELAWARE.

## PROPELLENT SMOKELESS-POWDER CHARGE.

1,393,623.

Specification of Letters Patent.

Patented Oct. 11, 1921.

No Drawing.

Application filed January 16, 1920. Serial No. 351,894.

To all whom it may concern:

Be it known that I, CLARENCE I. B. HENNING, a citizen of the United States, and a resident of Wilmington, in the county of 5 New Castle and State of Delaware, have invented a certain new and useful Propellant Smokeless-Powder Charge, of which the following is a specification.

This invention relates to a charge of progressive burning smokeless powder of the surface treated type, and comprises a charge in which nitrocellulose powder of the above mentioned character is associated with a supplementary priming charge consisting essentially of an easily ignitable propellant, such as black powder.

While all smokeless powders are progressive burning, the term "progressive burning powders" has in recent years been applied 20 to powders of the surface treated type which are extensively used in military rifles. In powder of this type the burning of the powder grain is regulated by treating the surface of the powder grain with a deterrent 25 material or a deterrent explosive, or a mixture of these, causing the outer layer of the powder to burn more slowly, which results in reduced pressure at the breech of the gun and does not unduly increase the pressure 30 along the bore of the rifle. As might be expected, surface treated powders are more difficult to ignite than non-surface treated powders but this difficulty in ignition has been largely overcome by the use of decidedly stronger primers. Thus, by the use 35 of decidedly stronger primers for the ignition of surface treated powders, ballistic results have been obtained very much in advance over ballistic results obtainable from 40 non-surface treated powders. In view of this fact that surface treated powders have been used quite successfully in this manner, it had not been realized that greater possibilities existed in connection with the use of 45 powder of this type.

I have discovered an improved method of ignition for progressive burning powders of the surface treated type which makes it possible to obtain ballistic results far in advance 50 of those which it is possible to obtain without using my invention. I have found that it is possible to obtain improved ballistic results by using for a charge of progressive powder of about 50 grains a supplementary

black powder priming charge of more than 55 one grain and in general from about two to five grains, in addition to the usual primer for the ignition of progressive burning powders of the surface treated type. More especially I have found that, by using a supplementary black powder priming charge in addition to the usual primer, it is possible to readily ignite progressive burning powders of the surface treated type which up to the present time have been impossible of ignition or very difficultly ignited by the usual primers alone, due either to the use of a particular surface treating material or a mixture of materials, or to the use of an excessive amount of surface treating material 60 thereby producing powder grains whose surfaces are difficult or impossible to ignite by means of the usual primers alone. Therefore, by being able to produce proper ignition of progressive burning powders of the 65 surface treated type, whose surfaces have been treated with a greater amount of deterrent material or deterrent explosive, or mixture of these, than heretofore used, I have obtained an improved propellant powder 70 giving remarkable ballistic results, as evidenced by a very decided reduction in pressure. It is, therefore, possible to obtain a very decided increase in the velocity of the projectile and at the same time with a pressure not exceeding the pressure given by the usual propellant powders and in a great 75 many cases with a still lower pressure. Further advantages of my invention are that the use of a propellant powder at such a low 80 pressure is accompanied by a decided reduction in the erosion because of the lower temperature at which the powder is consumed. In addition, there is decided reduction in 85 muzzle flash.

My invention may be illustrated by the following example:—

The powder used may be made according to the usual processes for making progressive burning powder of the so-called surface-treated type. For example, sufficient nitrocellulose to give 100 parts by weight of nitrocellulose, which may be a mixture of nitrocellulose soluble in ether-alcohol with nitrocellulose relatively insoluble in 100 ether-alcohol, or may be soluble nitrocellulose alone, is dehydrated with ethyl alcohol 105 of approximately 95% strength by volume

by means of a dehydrating press in order to displace the water. The excess alcohol is removed from the nitrocellulose, leaving about 33½ parts, by weight, of the alcohol in the dehydrated nitrocellulose. To this is added approximately 66½ parts by weight of ethyl ether in a suitable mixing machine, preferably provided with brine refrigeration. To the nitrocellulose and solvent in the mixer there may be added one-half or more parts of diphenylamin or other stabilizer, together with graphite, powdered metals, nitrocompounds, etc., in varying amounts. The composition is thoroughly mixed and colloided, which operation in the mixer requires about one-half hour or more, depending on the efficiency of the mixer. After thoroughly mixing, the colloided composition is formed into preliminary blocks by means of a press. These blocks are then pressed in the so-called finishing press and the composition pressed through dies into strings, which strings are granulated by means of a cutting machine. The granulated powder is then placed for one or more days in solvent recovery apparatus to recover the alcohol and ether, and then dried in water or air to reduce the solvent remaining in the powder to a low amount. The powder is then surface treated with a deterrent material such as dimethyldiphenylurea or a deterrent explosive such as dinitrotoluene or a mixture of these two or other ingredients. The details of this surface treating process, which forms no part of the present invention, are described in U. S. Patents Nos. 1,310,848, 1,312,463 and 1,313,459. The black powder which I prefer to use is of the composition generally used for black sporting powder and of approximately the following composition:—

74.0% potassium nitrate,  
10.4% sulfur,  
15.6% charcoal.

However, I do not limit myself to any particular composition of black powder as it is obvious that I would use that composition which by tests gives the best results and likewise that granulation which by tests is found most suitable for the particular purpose desired. This supplementary priming charge is then mixed with the progressive powder grains; or it may be placed in the base of the shell; in any case the supplementary charge should be so associated with the progressive burning powder as to be in direct contact therewith.

Nitrocellulose powder grains prepared as described in the first part of the above example, but before surface treatment, gave in the .30/06 Springfield rifle, with the regular U. S. Government primed shell and with the 180-grain bullet an instrumental velocity at 78-feet of 2,481 feet per second, with a mean pressure of 48,950 pounds per square

inch, using a weight of charge of 42.6 grains. A portion of the same powder surface treated with 6 parts of dimethyldiphenylurea could not be ignited by means of the usual primer but on the addition of three grains of FFg black powder gave with a weight of charge of 51.0 grains a mean instrumental velocity of 2,418 feet per second, with a mean pressure of only 35,200 pounds per square inch.

I do not limit myself to the use of black powder or to the use of black powder containing saltpeter as many nitrate mixtures will give the same improved ignition of progressive burning powders of the surface-treated type as the black powder composition given above.

Instead of black powder or nitrate mixtures I may use nitrocellulose powder grains, nitrocellulose-nitroglycerin powder grains, or powder grains of the semi-smokeless type, that is, a mixture of black powder ingredients, sulfur, charcoal and saltpeter, with nitrocellulose or ground nitrocellulose powders. In fact I may use any easily ignitable propellant such as might be used in small arms and ordnance, as a supplementary priming charge to the usual primer in order to obtain better ignition of the more difficultly ignited progressive burning powders of the surface-treated type.

I claim:

1. A propellant charge comprising a progressive burning nitrocellulose powder of the surface treated type associated with a supplementary priming charge consisting essentially of an easily ignitable propellant powder.
2. A propellant charge comprising a progressive burning nitrocellulose powder of the surface treated type intimately mixed with a supplementary priming charge consisting essentially of an easily ignitable propellant powder.
3. A propellant charge comprising a progressive burning nitrocellulose powder of the surface treated type associated with a supplementary priming charge containing sulfur, charcoal, and potassium nitrate.
4. A propellant charge comprising nitrocellulose powder grains carrying a deterrent material at their surface, associated with an easily ignitable propellant powder.
5. A propellant charge comprising 50 parts of nitrocellulose powder grains carrying a deterrent material at their surface, associated with from about 2 to 5 parts of an easily ignitable propellant powder.
6. A propellant charge comprising nitrocellulose powder grains carrying a deterrent material at their surface, associated with a supplementary priming charge containing sulfur, charcoal, and potassium nitrate.
7. A propellant charge comprising nitrocellulose powder grains carrying a deterrent

- material at their surface, associated with a supplementary priming charge containing sulfur, charcoal, nitrocellulose, and potassium nitrate.
- 5 8. A propellant charge comprising nitrocellulose powder grains impregnated with a deterrent material, associated with a relatively small amount of a propellant powder containing sulfur, charcoal, and potassium nitrate.
- 10 9. An explosive composition comprising a mixture of about 50 parts of progressive burning smokeless powder of the surface treated type with from about 2 to 5 parts of
- 15 a powder containing sulfur, charcoal, and potassium nitrate.
- 20 10. An explosive composition comprising a mixture of about 50 parts of progressive burning smokeless powder of the surface treated type with from about 2 to 5 parts of a powder containing sulfur, charcoal, and potassium nitrate in the proportions of about 2 parts sulfur, 3 parts charcoal, and 15 parts potassium nitrate.
- 25 11. An explosive composition comprising a mixture of about 50 parts of progressive burning smokeless powder of the surface treated type with from about 2 to 5 parts of a powder containing sulfur, charcoal, nitrocellulose, and potassium nitrate.
- 30 12. A propellant charge comprising nitrocellulose powder grains carrying at their surface a deterrent explosive, associated with a supplementary priming charge consisting essentially of an easily ignitable propellant powder.
- 35 13. A propellant charge comprising nitrocellulose powder grains carrying at their surface a deterrent explosive, associated with a supplementary priming charge consisting essentially of sulfur, charcoal, and potassium nitrate.
- 40 14. A propellant charge comprising nitrocellulose powder grains carrying at their surface a deterrent explosive, associated with a supplementary priming charge consisting essentially of sulfur, charcoal, nitrocellulose, and potassium nitrate.
- 45 15. A propellant charge comprising nitrocellulose powder grains carrying at their surface a deterrent explosive, associated with a supplementary charge consisting essentially of nitrocellulose-nitroglycerin powder grains.

In testimony whereof I affix my signature. 55  
CLARENCE I. B. HENNING.